

[54] COMPOSITE WOODWIND REED

2,296,737 9/1942 Peterson ..... 84/383

[75] Inventor: John G. Backus, Palos Verdes Estates, Calif.

Primary Examiner—Richard B. Wilkinson

[73] Assignee: University of Southern California, Los Angeles, Calif.

Assistant Examiner—V. W. Miska

[22] Filed: Nov. 6, 1972

Attorney—Ford W. Harris, Jr. et al.

[21] Appl. No.: 303,700

## [57] ABSTRACT

[52] U.S. Cl. .... 84/383, 84/380

A composite woodwind reed including a body portion having a butt end and including a tapered vamp portion terminating in a tip end. Embedded in the reed are laterally spaced, longitudinal ribs at least some of which extend substantially from the butt end of the reed to the tip end thereof. A low density filler material fills the spaces between the stiffening ribs, the filler material comprising hollow bodies having diameters of a few thousandths of an inch and embedded in plastic. The upper and lower sides of the reed are covered by plastic coatings bonded to the body portion and the vamp portion.

[51] Int. Cl. .... B26d 5/42

6 Claims, 6 Drawing Figures

[58] Field of Search .... 84/383, 380, 381, 84/382

## [56] References Cited

## UNITED STATES PATENTS

|           |         |          |              |
|-----------|---------|----------|--------------|
| 1,779,522 | 10/1930 | Widmayer | ..... 84/383 |
| 3,165,963 | 1/1965  | Burns    | ..... 84/383 |
| 2,919,617 | 1/1960  | Brilhart | ..... 84/383 |



PATENTED SEP 18 1973

3,759,132

FIG. 1.



FIG. 2.



FIG. 3.



FIG. 4.



FIG. 6.



FIG. 5.



## COMPOSITE WOODWIND REED

## BACKGROUND OF THE INVENTION

The present invention relates in general to reeds for single or double reed woodwind instruments and, more particularly, to a synthetic reed for such instruments.

The problem of making well behaved reeds for woodwind instruments is centuries old. It has long been the custom to use as reed material a species of cane, *Arundo Donax*, which is common in Europe, but may also be grown elsewhere. Unfortunately, this material suffers from the disadvantage common to all naturally grown materials, which is unpredictability. No two pieces of cane are alike, and reeds made to identical dimensions will consequently play differently. To get a 15 reed that plays well is then a matter of altering the contours of a piece of cane by filing, scraping, sanding, and the like, until either it plays properly, or must be discarded. Quite a bit of folklore has grown up around the art of fashioning reeds.

In recent years, there have been numerous attempts to make reeds out of plastics of various kinds. Since plastics can be made to quite uniform specifications, reeds made of such materials should behave alike when made to the same dimensions. Unfortunately, plastic reeds have met with practically no acceptance by woodwind players. The tone produced by them is generally harsh and not as musically satisfactory as the tone produced by a good cane reed. The reason for the unsuitability of plastics is that its properties, such as elastic modulus and density, are much different from those of cane, and, until recently, no one knew what the properties of the reed material should be.

As a result of investigation of the properties of cane reeds, a number of factors were qualitatively isolated, and some important properties quantitatively measured. The Young's modulus for reed cane varies widely, but normally lies in the range of 700,000 to 2,000,000 pounds per square inch, and the density, when wet (which is the way it is used) ranges from about 0.8 to 1.0 grams per cubic centimeter. Common plastics, by contrast, have a Young's modulus of 200,000 to 500,000 pounds per square inch, and a density, wet or dry, of 1.3 to 2.0 grams per cubic centimeter. Given these differences, it is not surprising that reeds made of ordinary plastics behave differently from cane reeds. For example, that portion of the reed inside a clarinet player's mouth has a natural frequency of its own which will lie above 2,500 cycles per second for cane, but which is less than 1,500 cycles per second for plastic. This difference has a great effect on the quality of the tone produced by the reed.

Reinforced plastics, e.g., combinations of resins with glass fibers, glass cloth, and the like, have also proven unsatisfactory. One reason is that the vibrating end of a clarinet reed, for example, must be shaved down to a thickness of 0.005 inch, or less, and most reinforced plastics lose too much of their strength when machined to this thinness.

As further background material, attention is directed to my U.S. Pat. No. 3,420,132, granted Jan. 7, 1969, which overcomes some of the problems of cane and plastic reeds, but not all of them.

## OBJECTS AND SUMMARY OF INVENTION

With the foregoing background in mind, the primary object of the invention is to provide a composite wood-

wind reed, for either single or double reed instruments, having a density and elasticity closely approximating those of natural cane reeds.

More particularly, an important object is to provide 5 a composite reed having a density of less than 1.2 grams per cubic centimeter at the vibrating tip portion, and specifically an over-all density in the range of 0.7 to 1.0.

Another important object is to provide a composite 10 reed having a Young's modulus greater than 700,000 pounds per square inch at the vibrating tip portion, and specifically a Young's modulus in the range of 1,000,000 to 2,000,000.

Still more particularly, an important object is to provide 15 a composite reed wherein the desired elasticity is supplied by longitudinal metallic ribs, which occupy a small fraction of the volume of the reed, and wherein the remaining volume is filled with a material of low density, the reinforcing and filler materials being so selected and proportioned that the desired over-all Young's modulus and density are achieved.

Summarizing the invention, it comprises a composite 20 woodwind reed including a body portion having a butt end and including a tapered vamp portion terminating in a tip end, the reed having embedded therein laterally spaced, longitudinal metallic ribs at least some of which extend substantially from the butt end to the tip end. At 25 least the vamp portion, and preferably both the body and vamp portions, include a low density filler material filling the spaces between the ribs.

Another important object of the invention is to provide 30 a composite woodwind reed having the characteristics set forth in the preceding paragraph.

Yet another object of importance is to provide 35 a composite woodwind reed wherein the aforementioned filler material comprises hollow plastic or glass bodies having diameters of a few thousandths of an inch and embedded in plastic.

Still another important object is to provide a construction 40 wherein the upper and lower sides of the reed are covered by plastic coatings bonded to the body portion and the vamp portion.

The foregoing objects, advantages, features and results of the present invention, together with various other objects, advantages, features and results which will be evident to those skilled in the woodwind reed art 45 in the light of this disclosure, may be achieved with the exemplary embodiment of the invention illustrated in the accompanying drawing and described in detail hereinafter.

## DESCRIPTION OF DRAWING

In the drawing:

FIG. 1 is a side elevational view of a clarinet mouthpiece equipped with the composite reed of the invention;

FIG. 2 is a side elevational view of the composite 60 reed of the invention;

FIGS. 3 and 4 are bottom and top plan views of the composite reed, respectively taken as indicated by the arrowed lines 3-3 and 4-4 of FIG. 2; and

FIGS. 5 and 6 are enlarged transverse sectional views 65 respectively taken as indicated by the arrowed lines 5-5 and 6-6 of FIG. 2 of the drawing.

### DETAILED DESCRIPTION OF EXEMPLARY EMBODIMENT OF INVENTION

Referring to the drawing, illustrated in FIG. 1 is a conventional clarinet mouthpiece 10 to which a composite reed 12 of the invention is secured in the usual manner by a clamp 14 having clamping screws 16. The reed 12 includes a body portion 18 having a butt end 20 and includes tapered vamp portion 22 terminating in a tip end 24. The reed 12 has a flat upper surface 26 seated against the under side of the mouthpiece 10, and the tip end 24 of the reed is disposed adjacent and spaced below the proximal end of the mouthpiece. The lower surface of the reed 12 is rounded in cross section, as best shown in FIG. 6.

The configuration shown for the reed 12 is typical of a clarinet reed. However, it will be understood that the invention is equally applicable to reeds for other single reed instruments, or for double reed instruments, which would have substantially different external configurations.

Considering the reed 12 in more detail now, it includes laterally spaced, longitudinal metallic ribs 30 at least some of which extend the full length of the reed. In the particular construction shown, all of the ribs 30 extend the full length. However, an alternative, not shown, is to provide ribs extending the full length, and additional ribs extending from the tip end 24 to or into the body portion 18.

The ribs 30 provide the reed 12 with the necessary stiffness and the desired elasticity. Preferably, they are made of magnesium, which has a reasonable Young's modulus, coupled with a low density.

In the body portion 18 of the reed 12, the ribs 30 are embedded in a solid plastic 32, the plastic being an epoxy or polyester resin, or the equivalent. The solid plastic 32 preferably extends more than half the length of the reed 12 from the butt end 20 thereof toward the tip end 24. For example, the solid plastic 32 may extend to the transverse line 34 of FIG. 3. In this area, the stiffening ribs 30 prevent the body portion 18 from warping.

Throughout at least the vamp portion 22 of the reed 12, the spaces between the ribs 30 are filled in with a low density filler material 36. If desired, the solid plastic 32 may be replaced by the same low density filler material 36, the latter thus extending the whole length of the reed 12. Preferably, this filler material comprises "Microballoons", which are tiny hollow plastic or glass spheres of diameters ranging from about 0.002 inch to 0.005 inch. These hollow bodies are pressed into the spaces between the ribs 30, and then are saturated with a mixture of catalyzed epoxy resin and acetone. The acetone is allowed to evaporate off, and the reed blank is then baked to harden the epoxy. (It will be understood that other binders may be used). By varying the relative proportions of epoxy and acetone, the resulting filler 36 can be made to have a density as low as 0.3 grams per cubic centimeter.

Upon completion of the foregoing, the reed blank is 60

machined smooth on the bottom to form the flat side which will lie against the under side or lay of the mouthpiece 10. To strengthen the structure for further machining of the curved side of the reed 12, a layer 38 of plastic is bonded to the flat surface, this being necessary since the filler 36 is quite fragile. For example, the coating 38 may be Mylar 0.0005 inch thick, cemented on with a polyester cement. The vamp surface is then machined to the proper configuration and dimensions, and another plastic film 40 is then bonded to this side to further strengthen the reed. Thereafter, the tip end 24 of the reed is trimmed to the proper shape.

The foregoing construction results in a reed 12 having a density and Young's modulus within the ranges hereinbefore specified, and, more particularly, results in a reed having the desirable characteristics of good cane reeds. The reed 12 plays well, with a good tone, and will play high notes freely, all of which are important features.

Although an exemplary embodiment of the invention has been specifically disclosed herein for purposes of illustration, it will be understood that various changes, modifications and substitutions may be incorporated in such embodiment, and that the invention may be incorporated in other embodiments, all without departing from the spirit of the invention as defined by the claims hereinafter appearing.

I claim as my invention:

1. A composite woodwind reed including a body portion having a butt end and including a vamp portion terminating in a tip end, said reed having embedded therein laterally spaced, longitudinal metallic ribs at least some of which extend substantially from the butt end of said reed to the tip end thereof, at least said vamp portion including a low density filler material filling the spaces between said ribs, the density of said filler material being small as compared to the density of said ribs.

2. A composite woodwind reed according to claim 1 wherein said filler material includes voids having diameters of a few thousandths of an inch and in plastic.

3. A composite woodwind reed as defined in claim 2 wherein the upper and lower sides of said reed are covered by plastic coatings bonded to said body portion and said vamp portion.

4. A composite woodwind reed having a butt end and a tip end and having embedded therein laterally spaced, longitudinal ribs at least some of which extend substantially from said butt end to said tip end, said reed including a low density filler material filling the spaces between said ribs, the density of said filler material being small as compared to the density of said ribs.

5. A composite woodwind reed according to claim 4 having a density of less than 1.2 grams per cubic centimeter at the tip portion.

6. A composite woodwind reed according to claim 4 having an over-all Young's modulus greater than 700,000 pounds per square inch at the tip portion.

\* \* \* \* \*